

## UNITED STATES PATENT OFFICE

2,647,035

DYEING OF TEXTILE MATERIALS USING  
ALKYLAMINE ALGINATE THICKENERS

William J. Cramer, Jr., and Harry W. Fritz, Jr.,  
Cumberland, Md., assignors to Celanese Corporation of America, New York, N. Y., a corporation of Delaware

No Drawing. Application June 30, 1951,  
Serial No. 234,654

12 Claims. (Cl. 8—59)

1

This invention relates to the dyeing of textile materials and relates more particularly to dyebaths and to a process for the dyeing of organic derivative of cellulose textile materials therewith.

It has previously been proposed to dye organic derivative of cellulose textile materials, such as fabrics and the like, with a dyebath containing a dyestuff dissolved in a mixture of water and a lower aliphatic alcohol. Using a dyebath of this type, it is possible to dye organic derivative of cellulose textile materials not only with dyestuffs that exhibit a good affinity for the said materials when applied thereto from aqueous dyebaths, but also with dyestuffs that exhibit little or no affinity when applied to the organic derivative of cellulose textile materials from aqueous dyebaths, such as, for example, acid, basic, direct cotton and mordant dyestuffs. By suitable selection of the dyestuffs, it is possible by the use of the alcohol-water dyebaths to obtain dyeings on organic derivative of cellulose textile materials that are extremely fast to washing and that are also highly resistant to light and acid fading.

In certain applications, it is essential that the dyebath have a relatively high viscosity to avoid any spread of the dyebath when it is applied to the organic derivative of cellulose textile materials. For example, in dyeing the said materials locally as by printing, stencilling or the like, substantially no spread of the dyebath must take place if sharp, clear prints are to be obtained. Similarly, in the over-all printing or pad-dyeing of the organic derivative of cellulose textile materials, it is frequently desirable substantially to eliminate any migration of the dyebath during the skying of the dyed materials to avoid the development thereon of a mottled appearance. The substances that have hitherto been commonly used for increasing the viscosity of or thickening aqueous dyebaths, such as gum arabic, gum tragacanth and the like, are not suited for the thickening of alcohol-water dyebaths in that they do not yield a thickened dyebath that has a uniform, smooth and stable consistency.

It is an important object of this invention to provide a thickened alcohol-water dyebath which will be free from the foregoing and other difficulties.

A further object of this invention is to provide an alcohol-water dyebath thickened with an alkylamine alginate.

Another object of this invention is to provide a process for the coloration of organic derivative of cellulose materials with an alcohol-water dyebath thickened with an alkylamine alginate.

2

Other objects of this invention will be apparent from the following detailed description and claims.

According to the present invention, a dyebath containing a dyestuff dissolved in a mixture of water and at least about 5% by weight, preferably between about 70 and 80% by weight, of a lower aliphatic alcohol is thickened by the addition thereto of an alkylamine alginate. The alcohol-water dyebaths thickened with the alkylamine alginate exhibit a uniform, smooth and stable consistency. In addition, they exhibit no tendency to foam, which foam may lead to the formation of spots on the dyed organic derivative of cellulose textile material. Moreover, the said dyebaths are easily and quickly prepared by adding an alkylamine alginate to the dyebath and stirring the same. After the dyeing of the organic derivative of cellulose textile material is effected, the alkylamine alginate may be readily removed from the dyed textile material by a simple scouring operation with hot water or a hot aqueous soap solution.

Examples of lower aliphatic alcohols that may be employed in preparing the dyebath of this invention include methyl alcohol, ethyl alcohol, normal propyl alcohol and isopropyl alcohol, as well as mixtures of these alcohols. In addition to the alcohol, the dyebath may contain inorganic or organic swelling agents for the organic derivative of cellulose material. Suitable inorganic swelling agents include, for example, the thiocyanates such as potassium thiocyanate, sodium thiocyanate and ammonium thiocyanate. Suitable organic swelling agents include, for example, di- and poly-alkylene glycols and their sulfur analogues such as diethylene glycol and thiodiglycol, tetrahydro-furfuryl alcohol, esters of hydroxy carboxylic acids such as ethyl lactate, and esters of di- or polyhydric alcohols or of di- or poly-alkylene glycols such as monoacetin, diacetin or triacetin.

Alkylamine alginates that may be added to the dyebath to thicken the same include, for example, diethylamine alginate, dipropylamine alginate and dibutylamine alginate. Depending upon the degree of thickening desired and the precise composition of the dyebath, there may be added to the dyebath from about 0.1 to 10% by weight of the alkylamine alginate; the lower concentrations of the alkylamine alginate serving to produce a dyebath suitable for pad-dyeing and over-all printing, and the higher concentrations of the alginate serving to produce a dyebath suitable for printing, stencilling and the like.

Dyestuffs that may be employed in compound-

ing the dyebath of this invention include, for example, Wool Fast Blue GL-C. I. 833, Azo-Rubinol 3GP-Pr. 412, Amacel Pure Scarlet III, Celliton Fast Blue AF, Pr. 227, Eosine Y-C. I. 768, Setacyl Direct Discharge Blue G, Amacel Rubine IX and Amacel Yellow CW. The dyestuff used should be free from sodium sulfate, commonly employed in standardizing the strength of dyestuffs, since the sodium sulfate tends to precipitate the alkylamine alginate.

The invention will now be described in connection with the dyeing of cellulose acetate which is commercially the most important organic derivative of cellulose material at the present time. It may, however, also be employed for the dyeing of other organic derivative of cellulose materials such as, cellulose propionate, cellulose butyrate, cellulose acetate propionate, cellulose acetate butyrate, ethyl cellulose and the like.

The following example is given to illustrate his invention further.

#### Example

In a mixture of 306 parts by weight of ethyl alcohol (95% by volume) and 125 parts by weight of water there is dissolved 5 parts by weight of Amacel Pure Scarlet III. The solution is placed in a stirrer and 12.5 parts by weight of dibutylamine alginate are sifted slowly into the solution with vigorous stirring and stirring is continued for 5 minutes after the addition of the alginate has been completed. A smooth non-frothing dyebath or paste is obtained which is of a consistency suitable for textile printing.

The thickened dyebath is heated to 45° C. and is printed onto a dry, scoured fabric formed of cellulose acetate yarns, following which the fabric is allowed to air dry for 10 seconds. The printed fabric is then can dried, soaped for 30 seconds in an aqueous solution containing 1 gram per liter of soap and maintained at 40° C., rinsed in hot water, extracted and dried. There is obtained a solid, well-penetrated, sharply defined print of good color value and the fabric exhibits no evidence of tendering in the printed area.

While our invention has been described in connection with the printing and dyeing of organic derivative of cellulose textile materials, it will be appreciated that the process of our invention may be employed for the printing or dyeing of films or foils having a basis of an organic derivative of cellulose.

It is to be understood that the foregoing detailed description is given merely by way of illustration and that many variations may be made therein without departing from the spirit of our invention.

Having described our invention, what we desire to secure by Letters Patent is:

1. A dyebath comprising a solution of a dyestuff in a mixture of water and at least about 5% by weight of a lower aliphatic alcohol, said dyebath being thickened with an alkylamine alginate selected from the group consisting of diethylamine alginate, dipropylamine alginate and dibutylamine alginate.

2. A dyebath comprising a solution of a dyestuff in a mixture of water and at least about 5% by weight of a lower aliphatic alcohol, said dyebath being thickened with from about 0.1 to 10% by weight of an alkylamine alginate selected from the group consisting of diethylamine

alginate, dipropylamine alginate and dibutylamine alginate.

3. A dyebath comprising a solution of a dyestuff in a mixture of water and from about 70 to 80% by weight of a lower aliphatic alcohol, said dyebath being thickened with from about 0.1 to 10% by weight of an alkylamine alginate selected from the group consisting of diethylamine alginate, dipropylamine alginate and dibutylamine alginate.

4. A dyebath comprising a solution of a dyestuff in a mixture of water and at least about 5% by weight of a lower aliphatic alcohol, said dyebath being thickened with dibutylamine alginate.

5. A dyebath comprising a solution of a dyestuff in a mixture of water and at least about 5% by weight of a lower aliphatic alcohol, said dyebath being thickened with from about 0.1 to 10% by weight of dibutylamine alginate.

6. Process for the coloration of organic derivative of cellulose materials, which comprises applying to the said materials a coloring medium comprising a solution of a dyestuff in a mixture of water and at least about 5% by weight of a lower aliphatic alcohol, said dyebath being thickened with an alkylamine alginate selected from the group consisting of diethylamine alginate, dipropylamine alginate and dibutylamine alginate.

7. Process for the dyeing of organic derivative of cellulose textile materials, which comprises applying to the said materials a dyebath comprising a solution of a dyestuff in a mixture of water and from about 70 to 80% by weight of a lower aliphatic alcohol, said dyebath being thickened with from about 0.1 to 10% by weight of an alkylamine alginate selected from the group consisting of diethylamine alginate, dipropylamine alginate and dibutylamine alginate.

8. Process for the dyeing of organic derivative of cellulose textile materials, which comprises applying to the said materials a dyebath comprising a solution of a dyestuff in a mixture of water and at least about 5% by weight of a lower aliphatic alcohol, said dyebath being thickened with dibutylamine alginate.

9. Process for the dyeing of organic derivative of cellulose textile materials, which comprises applying to the said materials a dyebath comprising a solution of a dyestuff in a mixture of water and at least about 5% by weight of a lower aliphatic alcohol, said dyebath being thickened with from about 0.1 to 10% by weight of dibutylamine alginate.

10. Process for the dyeing of cellulose acetate textile materials, which comprises applying to the said materials a dyebath comprising a solution of a dyestuff in a mixture of water and at least about 5% by weight of a lower aliphatic alcohol, said dyebath being thickened with an alkylamine alginate selected from the group consisting of diethylamine alginate, dipropylamine alginate and dibutylamine alginate.

11. Process for the dyeing of cellulose acetate textile materials, which comprises applying to the said materials a dyebath comprising a solution of a dyestuff in a mixture of water and from about 70 to 80% by weight of a lower aliphatic alcohol, said dyebath being thickened with from about 0.1 to 10% by weight of an alkylamine alginate selected from the group consisting of diethylamine alginate, dipropylamine alginate and dibutylamine alginate.

12. Process for the dyeing of cellulose acetate textile materials, which comprises applying to the said materials a dyebath comprising a solution of a dyestuff in a mixture of water and at least about 5% by weight of a lower aliphatic alcohol, said dyebath being thickened with from about 0.1 to 10% by weight of dibutylamine alginic acid.

WILLIAM J. CRAMER, JR.  
HARRY W. FRITZ, JR.

## References Cited in the file of this patent

## UNITED STATES PATENTS

| Number      | Name         | Date          |
|-------------|--------------|---------------|
| 5 2,158,486 | Preble ----- | May 16, 1939  |
| 2,514,410   | Olpin -----  | July 11, 1950 |

## OTHER REFERENCES

- American Dyestuff Reporter for November 28, 1938 (article by Cate), pages 716 to 721.  
10 Melliand Textilberichte for March 1950 (article by Schmidt), pages 194 to 196.